

# UNITED STATES PATENT OFFICE.

GEORGE W. PRIEST, OF WILMINGTON, DELAWARE, ASSIGNOR TO E. I. DU PONT DE NEMOURS & COMPANY, OF WILMINGTON, DELAWARE, A CORPORATION OF DELAWARE.

## PROCESS FOR PRODUCING LINOLEUM AND PRODUCT THEREOF.

1,381,737.

Specification of Letters Patent. Patented June 14, 1921.

No Drawing. Original application filed August 8, 1917, Serial No. 185,016. Divided and this application filed September 25, 1918. Serial No. 255,588.

To all whom it may concern:

Be it known that I, GEORGE W. PRIEST, of Wilmington, in the county of New Castle and in the State of Delaware, have invented 5 a certain new and useful Improvement in Processes for Producing Linoleum and Product Thereof, and do hereby declare that the following is a full, clear, and exact description thereof.

10 My invention relates to plastic compositions containing polymerized coumarone, and to a process of making such compositions.

15 The particular object of my invention is to provide a process of advantageous character for making linoleum compositions, particularly linoleum cements, and the product thereof.

20 Further objects of my invention will appear from a detailed description thereof contained hereinafter.

I have found that when a previously oxidized oil is ground together in any suitable machine, as for example a machine containing 25 friction rolls, with a polymerized product of the coumarone or indene group of compounds at a temperature of 100° C. or below a material is obtained which has characteristics as to its consistency, combining 30 qualities, solubility, etc., which make it more useful as a cement than in the case where the polymerized product of the coumarone or indene group of compounds is added to the oil before or while heating or oxidizing 35 the same.

While my invention is capable of being carried out in many different ways, I shall describe only one example thereof herein-after.

40 In order to carry out my process I may oxidize two parts of linseed oil in any suitable manner as for example by the application of heat and air so as to produce a jelly-like material. The thus obtained material 45 having a solid consistency is allowed to cool and I then mix therewith one part of a polymerized product of the coumarone or indene group of compounds and grind the same together at a temperature of 100° C. 50 or below thus producing a composition which is elastic, adhesive, coherent and light in color.

This composition may be used for linoleum cement by mixing with suitable proportions of pigment, ground cork or woodmeal, as 55 for example:

|                                   |          |
|-----------------------------------|----------|
| Linseed oil coumarone composition | 50 parts |
| Pigment                           | 20 parts |
| Ground cork or woodmeal           | 50 parts |

60 and applying to a fabric by means of pressure. The material may also be used for cementing materials of other kinds together and on fabrics of all kinds.

65 While I have described my invention above in detail, I wish it to be understood that many changes may be made therein without departing from the spirit of the same.

70 This application is a division of my application Serial No. 185,016, filed August 8, 1917.

I claim:

1. The process which comprises mixing 75 together an oxidized oil and a polymerized product of the coumarone or indene group of compounds at a temperature not above 100° C.

2. The process which comprises mixing 80 together an oxidized oil and a polymerized product of the coumarone or indene group of compounds and grinding them together between rolls.

3. The process which comprises mixing 85 together an oxidized oil and a polymerized product of the coumarone or indene group of compounds at a temperature not above 100° C. and grinding them together between rolls.

90 4. The process which comprises mixing together oxidized linseed oil and a polymerized product of the coumarone or indene group of compounds at a temperature not above 100° C.

95 5. The process which comprises mixing together oxidized linseed oil and a polymerized product of the coumarone or indene group of compounds and grinding them together between rolls.

100 6. The process which comprises mixing together oxidized linseed oil and a polymerized product of the coumarone or indene group of compounds at a temperature not

- above 100° C. and grinding them together between rolls.
7. A composition of matter comprising an oxidized oil having a solid consistency mixed with a polymerized product of the coumarone or indene group of compounds.
8. A composition of matter comprising an oxidized oil mixed and ground together with a polymerized product of the coumarone or indene group of compounds.
9. A composition of matter comprising oxidized linseed oil having a solid consistency mixed with a polymerized product of
- the coumarone or indene group of compounds.
10. A composition of matter comprising oxidized linseed oil mixed and ground together with a polymerized product of the coumarone or indene group of compounds.

In testimony that I claim the foregoing I have hereunto set my hand.

GEORGE W. PRIEST.

Witnesses:

G. D. HOPKINS,  
STANLEY L. ABRAMS.